

July 26, 1932.

E. D. VANCE

1,868,931

PROCESS FOR MAKING ABRASIVE ARTICLES

Filed May 19, 1930

FIG. 1



FIG. 2



INVENTOR

Edward D. Vance

BY

Staley & Welch

ATTORNEYS

## UNITED STATES PATENT OFFICE

EDWARD D. VANCE, OF SPRINGFIELD, OHIO, ASSIGNOR TO THE SAFETY GRINDING WHEEL & MACHINE COMPANY, OF SPRINGFIELD, OHIO, A CORPORATION OF OHIO

## PROCESS FOR MAKING ABRASIVE ARTICLES

Application filed May 19, 1930. Serial No. 453,626.

My invention relates to improvements in abrasive articles and particularly to grinding wheels.

Abrasive articles such as grinding wheels have been made with various granular substances with different kinds of binders. One of the most common forms is what is known as vitrified or silicate wheels in which the granular material such as emery or carbon 5 rindum, etc., is bound together by silicate binders which when baked at a proper temperature forms a porous substance consisting of the granular elements held together by the binder which is more or less solidified.

It has also been the practice to supply these porous wheels when desired with an auxiliary binder such as synthetic resin, shellac and the like. These supplemental binders are applied to the porous articles by dipping the 20 wheel or other article into a liquid solution of the particular substance which makes up the auxiliary binder and afterwards allowing it to properly set, preferably by the application of heat.

Considerable difficulty has been experienced in obtaining a wheel of uniform texture with a supplemental binder by the methods heretofore employed as the supplemental binder in liquid form will change its position in the porous substance before it is properly set and a portion of it will escape through the pores so as to leave the article in an unbalanced condition or with some of the pores completely filled and others only partially filled with the liquid binder.

To overcome these difficulties I have designed a process by which the article is uniformly filled and the liquid properly maintained in the pores until the supplemental binder is completely set by the application of heat or otherwise.

In carrying out this process I take an ordinary porous abrasive article or grinding wheel which has been formed by the vitrifying or other process and coat the same on all of the outer surfaces but one with a quickly setting cement and then applying the supplemental binder in liquid form to the uncoated side until all the pores are completely

filled and usually with an excess of the material on the uncoated side.

When synthetic resin and similar substances are used as an auxiliary binder the article so impregnated is maintained in an upright position or in the position in which the uncoated side is at the top and the same is then inserted into a suitable kiln where it is heated to the proper temperature to completely set the auxiliary binder or change it into a hard tough supplemental bond.

After the supplemental binder has thus been treated the article is removed from the kiln and the outer covering of cement which retains the supplemental binder in place before the application of heat and the surplus material on the uncoated side of the article is then removed by a process of dressing which in the case of wheels would consist in supporting the wheel in a proper position and with proper tools removing the surplus material and the outer coating.

Wheels thus treated it has been found in practice have a more perfect supplemental binder and a completely homogeneous mass and with a supplemental binder which is uniform throughout thus making a perfectly balanced wheel or other article and also much stronger than when the supplemental binder is applied by dipping or otherwise.

In the drawing attached thereto:

Fig. 1 is a plan view of a wheel to which the outer coating of cement has been applied and in a position to receive the liquid supplemental binder.

Fig. 2 is a cross section of the same.

In these figures, 1 represents the porous wheel or other article and 2 a coating of cement around the periphery and the bottom of the wheel and also the sides of the openings 3 which ordinarily extend through the center of a grinding wheel.

For coating the sides and periphery of this wheel to stop the pores to prevent the leakage of the liquid binder I use any suitable cement preferably one which will stand the temperature of baking where synthetic resin and similar substances are employed for the auxiliary binder. Air drying cement such as Portland cement or suitable forms of clay

cement may be used. I have very successfully used a commercial cement under the trade-name "Sair Set Cement."

5 Having thus described my invention, I claim:

1. The process of applying a supplemental binder to a porous abrasive article which consists in coating such article on all its sides except one with a pore stopping cement, applying said supplemental binder in a liquid form to the uncoated side of said article until all the pores are uniformly filled, retaining the article in the position in which the liquid binder is applied until it has properly and permanently set and then removing the outer pore stopping covering and the surplus binding material.
- 10 2. The process of applying a supplemental binder to abrasive articles formed of a porous material which consists in applying a temporary quickly setting covering which will stop the pores on all the sides of said article except one, applying a supplemental binder in liquid form to the uncoated side of said article, retaining the same in the position in which the liquid is applied and subjecting the same to heat in the same position until the binder is completely and permanently set and then removing the outer cover and the surplus material.
- 15 3. The process of making an abrasive wheel which consists in applying to a vitrified or other porous wheel a coating of air drying cement on all the surfaces of said wheel except one, applying a liquid supplemental binder to the uncoated side, subjecting the article to heat to permanently set the supplemental binder and thereafter removing the pore stopping coating and surplus binder from the sides and periphery of the wheel.
- 20 4. The process of applying a supplemental binder in liquid form to a porous abrasive article which consists in coating the major portion of such article with a covering impervious to the binder, applying such supplemental binder to the exposed portion of such article, and removing the outer covering after the binder has set.
- 25 5. The process of applying a supplemental binder in liquid form to a porous abrasive article which consists in coating the major portion of such article with a covering impervious to the binder and of a character to resist heat sufficient to set the binder, applying the liquid binder to the exposed portion of said article, then setting the same by heat and thereafter removing the covering.
- 30 In testimony whereof, I have hereunto set my hand this 15th day of May, 1930.

EDWARD D. VANCE.